

Oct. 16, 1928.

1,687,815

H. E. WETHERBEE

METHOD OF TREATING AND FORMING ARTIFICIAL FUEL

Filed April 13, 1926



INVENTOR:

*Herbert E. Wetherbee,*

BY

*Herbert E. Wetherbee*  
ATTORNEY.

Patented Oct. 16, 1928.

1,687,815

## UNITED STATES PATENT OFFICE.

HERBERT E. WETHERBEE, OF CLEVELAND, OHIO, ASSIGNOR OF ONE-THIRD TO RICHARD F. GRANT AND ONE-THIRD TO HOWARD M. HANNA, BOTH OF CLEVELAND, OHIO.

### METHOD OF TREATING AND FORMING ARTIFICIAL FUEL.

Application filed April 13, 1926. Serial No. 101,639.

My invention relates to improvements in methods of treating and forming artificial fuel, and to the resultant fuel produced thereby; the object of my invention being to produce a fuel from small sizes of fuel materials such as anthracite or bituminous coals, lignite, or other carbonaceous materials. Primarily, my invention thus far has been applied to coalescing various small sizes of anthracite in order to produce a fuel commercially available for domestic and other uses.

The present invention is not concerned with the particular mode of coalescing or of briquetting the fuel, as commercially practiced, but relates primarily to the preliminary step or treatment of the subdivided fuel whereby the binding material may expeditiously and cheaply be applied to the fuel particles in order to produce a fuel that will be satisfactory, not only for combustion purposes even after a considerable lapse of time, but will be adapted for transportation. The requirements for these purposes are distinctly different, in that a binding material affording the requisite toughness for rough handling of the completed product, may not serve to retain the particles in their coalesced state when subjected to the intense heat of the furnace, and the converse is equally true.

In the development of the art, many binding materials have been suggested and a wide variety thereof has actually been used in the briquetting of fuels, but these present a wide and varying range as to their cost, and more or less unsatisfactory characteristics in applying such binding material to the subdivided fuel.

Accordingly, my invention essentially has been directed toward the ready and economical application of the binding material to the fuel particles, which advantageously may be of varying sizes produced in the mining of anthracite or other coals. This improvement, then, is based upon the application of any suitable binding material to the fuel particles by means of a filming carrier, and one preferably adapted to displace a moisture or water film upon the surfaces of the particles. Thus, an oil associated with a binder otherwise difficult of application to carbonaceous materials, may be employed as a carrier whereby a wide range of binding materials

may be evenly applied with the oil to the fuel particles. By this I do not mean that my invention necessarily is limited to the use of a 55 filming oil, since other fluids may be used as a filming carrier for the binder.

Hitherto, marked difficulty has been experienced in all briquetting processes with which I am familiar in getting a suitable binding material into sufficiently intimate contact with the subdivided fuel or carbonaceous material preparatory to briquetting the same. Usually this requires a thorough drying of the carbonaceous material before the binder 60 is applied, in order to remove the water coating or moisture and thus permit the binder to make contact therewith. Obviously, such drying operation requires the equipment of an extensive plant therefor, and adds mate- 65 rially to the cost of the product.

My experience has shown that a relatively small amount of suitable binding material, evenly distributed over the particles of subdivided fuel and in intimate contact therewith will suffice to bind the fuel material into a commercial briquette upon subjecting the same to pressure. The difficulty with present commercial processes has been that the methods employed do not evenly distribute 70 the binder over the fuel material, thereby requiring an excessive amount of binder and unduly increasing the cost of the product.

Accordingly, I have directed my efforts toward perfecting a method which will, first, 75 bring the selected binding material into intimate contact with the subdivided fuel without drying the same, and, second, a method which will apply such binding material cheaply, evenly, and quickly over the particles of 80 the fuel material, thereby effecting definite savings in operating and material costs.

The spreading action of oils on water is well known, even with respect to oils of marked viscosity. Moreover, since carbonaceous material has a distinctly greater adhering power for oil than for water, the water adhering to immersed carbonaceous material will be displaced by an adherent film of oil. This principle I have availed of to obtain a carrier for 85 any suitable binding material, which preferably is associated or mixed with the oil.

In addition to the aforesaid spreading action of oil upon water, I also have availed of

the results of thorough agitation of the liquids and fuel material, whereby the oil and binding material are broken up into exceedingly small globules and distributed throughout the immersed fuel material, with the result that the filming or coating operation progresses rapidly through the immediate displacement of the surface covering of water upon the particles of the fuel material by the carrier and binder. Thus, it is rendered commercially practicable, and at normal temperature, to distribute a substantially uniform film of oil and binder, or of a dissolved binding material, by agitation of the subdivided carbonaceous or fuel material in water to which the carrier and binder have been added.

The range of possible carriers and associated binders, obviously is considerable and I cannot attempt herein to furnish any adequate or exhaustive list. Nevertheless, I have selected some typical examples of applying varying amounts of binding material to subdivided fuel by means of suitably selected and treated carriers, solvents or semi-solvents. As indicated above, the binding material should possess the qualities of producing a strongly adherent briquette of firm, tough texture, which will stand transporting to great distances, remain stable for months, and will not crack or crumble in firing the same. Such carriers and binders may be applied to the fuel material in two ways—

First: By mixing the binding material or materials with the oil or fluid carrier before agitating the same with the subdivided fuel and water, as indicated above, in which case the oil film formed on the carbonaceous material carries with it the associated binding material or materials.

Second: By first forming the oil film on the carbonaceous material by suitable agitation, then draining off the excess water and treating the oil filmed carbonaceous material in a bath containing the selected binding material or materials. In this case the binding material will be taken out of the bath by the adherent action of the oil film for the binding material.

It should be observed that many oils, per se, possess marked binding characteristics, while serving equally well as carriers, and that other liquids not classed as oils have the requisite adherent quality for carbonaceous material to serve as carriers, some of which may be used as solvents for binding materials and the resultant solution may thus be utilized in the same manner as an oil.

While I shall herein instance the use of suitable oils, solvents and binding materials for practicing my invention, I do not wish to be understood as necessarily limiting the same thereto, since my improvement contemplates the use of any suitable carrier in association or admixture with binding material or mate-

rials, or any suitable fluid binder of slight or negligible miscibility with water, or any suitable binder dissolved in a suitable fluid carrier, any of which will produce a potentially adherent film under the conditions of subjecting the immersed carbonaceous material thereto, without artificial drying, treating the same and briquetting or coalescing the fuel product.

I may also call attention to the difficulty which has heretofore been experienced in using varying sizes of carbonaceous material, coarser than the so-called anthracite culm, for briquetting, because proper adhesion of these varying and irregular sizes could not be obtained satisfactorily, and such efforts as have been made along these lines resulted in a fuel that was commercially unsatisfactory, whereas, under my improved procedure herein described, this difficulty is completely and satisfactorily overcome.

I have shown somewhat diagrammatically in the accompanying drawings one means for practicing the methods herein described, wherein:

Figure 1 is an end elevation of a rotatable cylinder or drum wherein the mixing and agitation may be effected;

Fig. 2 is a side elevation thereof;

Fig. 3 is a transverse section on line 3—3, Fig. 2, generally indicating the fuel and water levels, and

Fig. 4 is a longitudinal section thereof on line 4—4, Fig. 1.

Throughout the several figures of the drawings I have employed the same character of reference to indicate similar parts.

In the somewhat diagrammatic showing herewith, the rotatable cylinder *c* is mounted on stub-shafts *s*, rotatably supported by the standards *s'* and actuated by the driven gear *g*. Within the cylinder there are provided a plurality of baffles *b* which are adapted to elevate the sub-divided fuel *f* above the level of the water *w* and its surface coating *a* of combined carrier and binding material, through which the fuel particles are permitted to fall as the cylinder is rotated.

The contents may be supplied to the cylinder by means of the chutes *c'* when the hand hole *h* is rotated to the upper position shown in Fig. 2; this opening thereupon being tightly closed to permit of the agitation of the contents by rotating the cylinder when it is fully charged. Obviously, upon such rotation, thorough agitation of the contents is effected, the subdivided fuel material *f* being carried up by the baffles and dropped through and agitated with the surface coating *a* of carrier and agglutinating material for the purpose of enabling the particles of fuel to make frequent and practically continuous contact with the filmed and small particles of oil distributed on and throughout the water. This serves to effect an even distribution of the

carrier and the associated binder or agglutinating material throughout the entire mass of the subdivided fuel.

It will be understood, of course, that the proportions in the drawing, and particularly, the stratum *a* of carrier and binding material, are merely illustrative, and do not represent operating conditions, relative quantities or volumes, and sizes of subdivided fuel or mechanical parts.

As formulae exemplifying the practice of my instant invention, I may state that with a given quantity of the finer breaker products of anthracite, comprising roughly a major imbedding content of culm and twenty per cent (20%) each of Nos. 1, 2 and 3 buckwheat, for example, I employ the various percentages by weight, of carrier and binding material or materials hereinafter indicated for producing briquettes of satisfactory strength and burning qualities. It should be explained, however, that no fixed proportions of the different sizes of anthracite are required, and that other fuel materials lend themselves equally well to the method of treatment for producing artificial fuels in accordance with my invention.

Premising the disclosure of a few typical formulae for employing associated carrier and binding materials, I may explain that the oxidizable or potentially solidifying oils afford a combined carrier and binding medium which impart toughness to the fuel product. Cheaper oils or carrier material, however, may be substituted when desirable, by selecting a suitable associated binding medium, usually with the attendant requirement of employing a larger percentage of the combined carrier-binder material.

As an example of a carrier-binder employing an oxidizing, agglutinating oil, one per cent (1%) by weight of a mixture comprising eighty per cent (80%) linseed oil and twenty per cent (20%) kauri paste, or twenty per cent (20%) rosin, in substitution for the latter, may be successfully employed in practicing my improvement.

Approximately two per cent (2%) by weight of a carrier-binder comprising thirty per cent (30%) gilsonite dissolved in seventy per cent (70%) of gasoline, likewise may advantageously be substituted for the above.

Approximately five per cent (5%) of a carrier-binder comprising twenty-five per cent (25%) light blending oil from coal tar distillation, thirty-seven and one-half per cent (37½%) blown asphalt, and thirty-seven and one-half per cent (37½%) heavy refined tar or 190° pitch, also is adapted for practicing my invention. This mixture most advantageously is applied to the fuel particles in a bath of water initially heated approximately to the boiling point.

Again the subdivided fuel may first be

filmed with one-half per cent (½%) by weight of linseed oil, after which the excess water may be drained off and displaced with a ten per cent (10%) solution of dextrine in water; both accompanied by agitation, whereby the oil film serves as an effective carrier for the binder in question.

It will be unnecessary to multiply these formulae, however, since it is sufficient to emphasize the need for employing a suitable carrier in small amounts for applying a binder or associated binding materials to the moistened subdivided fuel evenly and quickly in order to coalesce or agglomerate the particles thereof when subjected to pressure.

The binding materials indicated in the foregoing examples not only are found to possess sufficient toughening qualities for transportation purposes, but said materials will burn approximately the same way as does the agglomerated fuel. In consequence, briquettes can be produced in accordance with my invention which are equally satisfactory for purposes of transportation and combustion, which is not the case where some classes of binders are used.

My instant process has the obvious advantages and economies of—

First—elimination of drying the carbonaceous material;

Second—even and continuous distribution of the binding material on the carbonaceous material in intimate contact therewith, thereby requiring the use of a minimum amount of binding material and saving the expense of additional and unnecessary binder required under other methods and processes.

Accordingly, the briquettes produced in accordance with my instant improvement are low in cost while satisfying every commercial requirement.

Having now described the preferred procedure for practicing my invention, I claim as new and desire to secure by Letters Patent, together with such modifications as to procedure, proportions and ingredients used, as may be supplied by one ordinarily skilled in the art, the following:

1. The herein described method of treating subdivided fuel materials preliminary to coalescing the same, which consists in subjecting a mass thereof in moistened condition to the action of a filming carrier and a binding material for the fuel, whereby the latter is evenly applied to the fuel particles, substantially as set forth.

2. In a method for treating subdivided fuel materials preliminary to coalescing the same, the step of subjecting the particles thereof to a filming material as a carrier for a binder and to an associated binding material adapted thereby evenly to coat the particles, substantially as set forth.

3. In a method for treating subdivided fuel

material preliminary to coalescing the same, the step of subjecting the particles thereof while in moistened condition to the action of a moisture-displacing carrier and to a binding material adapted thereby to coat the particles of fuel, substantially as set forth.

4. In a method for treating subdivided fuel materials preliminary to coalescing the same, the step of subjecting the particles thereof 10 while in moistened condition to the action of filming oil and to a binding material adapted thereby evenly to coat the particles of fuel, substantially as set forth.

5. The method of producing artificial fuel 15 which consists in immersing subdivided carbonaceous material in water, adding to the water a moisture-displacing filming oil and binding material carried by the oil, agitating the carbonaceous material with the oil-carrier 20 and binder to produce a substantially uniform adherent film upon the particles of carbonaceous material, draining off the excess water, and subjecting portions of the mass to pres-

sure inducing adhesion thereof, substantially as set forth.

6. In a method for treating comminuted fuel materials preliminary to briquetting the same, the subjection of the particles thereof while in an aqueous bath to the action of a 25 filming carrier and to a binding material, together having negligible miscibility with water, substantially as set forth.

7. The method of producing artificial fuel which consists in immersing sub-divided carbonaceous material in an aqueous bath, adding thereto an adherent oil content with other binding material which together have negligible miscibility with water, agitating the carbonaceous material therewith, draining off the excess water, and subjecting portions 30 of the carbonaceous mass to pressure sufficient to induce adhesion of the particles, substantially as set forth.

In testimony whereof I do now affix my signature.

HERBERT E. WETHERBEE.